

No. 710,882.

Patented Oct. 7, 1902.

S. NORTON.

ART OF MOLDING SLAG.

(Application filed Dec. 6, 1901.)

(No Model.)



Inventor

Sheldon Norton.

Witnesses

H. G. Amer.  
A. G. Chapman.

By Victor J. Evans

Attorney

# UNITED STATES PATENT OFFICE.

SHELDON NORTON, OF CATASAUQUA, PENNSYLVANIA, ASSIGNOR OF  
ONE-HALF TO W. L. SIMS, OF CATASAUQUA, PENNSYLVANIA.

## ART OF MOLDING SLAG.

SPECIFICATION forming part of Letters Patent No. 710,882, dated October 7, 1902.

Application filed December 6, 1901. Serial No. 84,920. (No model.)

*To all whom it may concern:*

Be it known that I, SHELDON NORTON, a citizen of the United States of America, residing at Catasauqua, in the county of Lehigh, in 5 the State of Pennsylvania, have invented new and useful Improvements in the Art of Molding Slag, of which the following is a specification.

My invention has relation to improvements 10 in the art of molding articles directly from molten furnace-slag; and the object is to produce directly from molten furnace-slag articles of forms, such as bricks, tiles, and ornamental faces and blocks.

15 I accomplish the object by taking the molten slag from the furnace where it emanates, then conveying it to a second furnace, where it is deposited in a crucible or other suitable receptacle within the combustion-chamber of 20 the second furnace, then introducing and incorporating earthy material in the slag, and then restoring the mixture to a fused condition and so maintaining it. The molten mixture is then poured from the crucible into 25 molds traveling in the combustion-chamber of the furnace and passing through an elongated annealing and solidifying flue of gradually-decreasing temperature and discharged at a point for removal.

30 I have illustrated in the accompanying drawing a form of furnace and apparatus by which the invention may be practiced. The furnace for maintaining the slag in molten condition and for annealing and in which 35 the forms become solidified in their passage through the extended portion or lengthened flue of the combustion-chamber is shown in longitudinal vertical section and the appliances and mechanisms in side elevation, and, 40 reference being had thereto, A designates a furnace, B the fuel-chamber, and C the combustion-chamber extended into a flue of such length that the molded articles may pass through a channel or area of gradually-de- 45 creasing temperature from point of deposition to the point of discharge and in the passage become gradually annealed and sufficiently solidified to be discharged at the outer end of the carrier. The stack rises from the 50 outer end of the lengthened flue of the combustion-chamber opening from an enlarged

room E, formed under the stock by the upwardly-inclined furnace-roof and the extension of the rear wall of the furnace, as shown. In the roof of the furnace, at the rear and adjacent to the bridge 1 of the furnace, is an opening 2, through which the molten slag is poured. This opening may be closed by any suitable closure, when desired.

F designates the slag-delivering tub. This 60 is mounted on trucks 3 4, mounted on a track 5. The trucks have substantial standards 6 rising therefrom, formed with bearings through them, in which the gudgeons 7 8 of a tub-ring 9 are journaled. In the tub-ring is 65 arranged the slag-tub F, as shown. Directly under the opening 2 in the combustion-chamber of the furnace A is the crucible G, mounted to turn and tip on bearings 10, and may be turned thereon by means exterior of the 70 furnace and connected thereto. Longitudinally arranged in the combustion-chamber of the furnace below the general line of draft is mounted a mold-carrier H. This comprises a drum 11, suitably mounted at a point below 75 and adjacent to the crucible G, and at the rear end of the flue, on a higher plane than the drum 11, is arranged another drum 12. On these drums is arranged a traveling endless carrier 14, extending on a line substantially 80 parallel with the roof of the flue and consisting of a series of links 15, arranged in endless succession on the drums and formed with molds designed to be filled with the material deposited from the crucible. At the end of 85 the carrier is arranged an inclined plate or way 16, on which the solidified forms are discharged from the carrier onto a car or truck 17 to be conveyed to a desired place.

While the described process may, as described, produce a brick or other form of slag article, the process embraces the introduction and incorporation in the fused slag contained in the crucible in the furnace of earthy material, as clay or its equivalent, and then again 95 subjecting the mixture to fusion preliminary to pouring it off into the molds.

The apparatus being substantially of the construction and arrangement described, the steps in the process are carried out as follows: 100 The molten slag is deposited in a ladle or tub at the smelting-furnace (or is run directly

therefrom) and poured into the crucible G in the combustion-chamber of the fuel-chamber 5 B. After the required quantity of slag has been supplied to the crucible the earthy material is added for the purpose of imparting toughness to the mixture. The mixture thus made is then again subjected to heat while in 10 the crucible to restore the fusion, which being accomplished it is poured from the crucible into the molds, which are carried on the endless carrier through the extended flue and in their course subjected to a gradually-de- 15 creasing temperature, so that by the time they reach the limit of the carrier they become annealed and sufficiently solidified to be discharged.

The introduction and incorporation of the 20 earthy matter are for the purpose of imparting toughness and to cause the slag to assume a vitreous quality. Coloring material may be introduced in the molten slag while in the process of its transportation from the smelt-

ing-furnace either in the tub or runner, or it 25 may be incorporated in the material while in the crucible, as may be deemed the better.

Having described my invention, what I claim is—

The improvement in the art of molding 30 slag consisting in pouring molten slag into a crucible heated to a fusing temperature to sustain the fusion, then mixing earthy material with the fused slag, then restoring the mixture to fusion, then pouring the fused mix- 35 ture into traveling molds, then continuing the movement of the filled molds through an elongated flue of gradually-decreasing tempera- ture to anneal and solidify them, and then dis- charging the molded articles from the carrier. 40

In testimony whereof I affix my signature in presence of two witnesses.

SHELDON NORTON.

Witnesses:

CHAS. N. ULRICH,  
ALEX. N. ULRICH.